# EUROPEAN PATENT APPLICATION

(11) **EP 0 015 090 A1**
(43) Date of publication of application: **03.09.1980**
(21) Application number: 80300326.8
(22) Date of filing: 05.02.1980
(51) Int. Cl.: D21H 3/68

(54) **Method of and composition for sizing and fire proofing paper and paper made by the method**

(30) Priority: 22.02.1979 GB 7906315
(71) Applicant: Coal Industry (Patents) Limited, London SW1X 7AE (GB)
(72) Inventor: Hodges, Newton John, Charlton Kings Gloucestershire (GB); Riemer, Pierce William Foster, Hucclecote Gloucestershire (GB); Singleton, Clive Anthony, Newent-on-Trent Nottinghamshire (GB)
(74) Representative: Wood, John Irwin (GB)

(57) **Abstract**

Unsized paper is treated with an aqueous composition having a pH from 7.8 to 8.2 and comprising 10 to 70 parts of a dissolved ionic fire retardant and 0.2 to 1 parts of an emulsified alkylketene dimer.
The time of treatment is such that the paper has a dry material loading of fire retardant of 10 to 50% and of water repellant of 0.4 to 1 %.
The method is of particular use with handsheet paper.

## Description

This invention relates to the treatment of a web of unsized paper with an aqueous composition of flame retardant salts and a sizing material to produce paper with good sizing, flame resistance and strength. The invention also relates to the composition used for the treatment of the unsized paper and the paper produced by the treatment.

It is known to treat paper to render it flame resistant. However, the materials that are applied are expensive and can reduce both the strength and water resistance of the final paper.

It has been proposed to render a paper both water and fire resistant. However, it is very difficult to achieve this because the addition to paper of fire retarding compounds usually decreases significantly the water resistance of the paper. Many methods have been proposed for preparing water and fire resistant paper and some of these are set out in British Patent No. 1 500 612, to the International Paper Company. It will be seen from this patent that there are many problems to be solved in finding a suitable process for preparing fire and water resistant paper. One of the major problems is that in many cases the fire retarding agent and the water repelling agent are incompatible.

Another problem is that most solutions used to fire - and water-proof paper are acidic. These solutions attack the processing rollers in a paper mill and therefore make it necessary for the rollers to be replaced or refurbished frequently. This clearly adds to the cost of the paper making process and reduces its efficiency.

It is an aim of the present invention to provide a paper-treating solution which contains a compatible fire retardant and water repellant, and which does not corrode processing rollers to any substantial extent.

According to a first aspect of the present invention there is provided an aqueous paper-treating solution comprising from 10 to 70 parts of an ionic fire retardant material and from 0.2 to 1 part of an alkylketene dimer, wherein the solution has a pH from 7.8 to 8.2, preferably 8.0.

The solution according to the present invention has the advantage that paper treated with it does not show any evidence of incompatibility of the components. There is no evidence of one or the other component being unabsorbed by the paper. Another advantage of the solution is that it is only mildly alkaline, so that it is unable to attack the processing rollers, thus enabling relatively cheap and efficient running of a paper processing plant. These advantages are obtained because of the careful control of the pH solution.

Preferably the alkylketene dimer is supplied as an aqueous emulsion containing about 6% of the alkylketene dimer. The emulsion may also contain a cationic starch as a protective colloid. An especially suitable emulsion, supplied by Hercules Powder Company Limited, is Aquapel (RTM) 360X. This has a total solids content of 7.6%,an alkylketene dimer content of 6%, specific gravity of 1.02 at 25⁰C, a viscosity from 25 to 100 centipoise at 25°C and a pH of 3.5 to 4.0.

The fire retardant material may be based on sulphates, phosphates, borates or mixtures thereof. Preferably the fire retardant material comprises from 45 to 55% diammonium hydrogen phosphate, the balance being ammonium sulphate.

The fire retardant material may contain small amounts, up to about 10% of impurities. Preferably up to 30 parts of it are present in the solution. For good fire resistance it is desirable to have at least 10 parts of the fire retardant material present. The amount of water used to make the solution will be selected so that sufficient solution is taken up by the paper being treated to give the appropriate loading of water repellent and fire .retardant on the paper. This can be easily determined experimentally by those skilled in the art. The solution may also contain wet strength agents and other additives used in the paper making industry. These are well known in the art. It is generally recommended to use a cationic retention aid with alkylketene dimer sizing agents.

According to a second aspect of the present invention there is provided a method of treating a web of paper to render it fire and water resistant, comprising treating the paper with a solution according to the first aspect of the invention and drying the paper, wherein the treatment is such that the dried paper has a dry loading of fire retardant from 10 to 50% and of water repellent from 0.4 to 1%.

To achieve the appropriate loading it is possible to vary the concentration of the solution, the time of treatment or both. It is envisaged that the treatment will take place in a continuous process and the concentration of the solution will have to be arranged in relation to the speed of a web of paper passing through a treatment bath.

According to a third aspect of the invention there is provided a water - and fire - resistant paper when made according to the method of the second aspect of the invention.

Water repellency is measured according to the Cobb test, which is _{BS} 2644/1955. This measures the amount of water in grams absorbed by one square metre of paper in one minute. Thus-a good water-repelling paper has a low Cobb value.

Untreated handheet paper has a Cobb value in excess of 100. Handsheet paper treated according to the invention has a Cobb value of from 20 to 60. Handsheet paper treated with the fire retardant material alone has a Cobb value of over 100. If the pH of the solution is allowed to drop to about 7.5 the Cobb value of the handsheet paper rises to above 70. Acceptable Cobb values for sized paper are below 60.

Fire retarding properties are measured by the Technical Association of Pulp and Paper Industry Standard Method T461m-48, (TAPPI test) which is also found as ASTM D 777-46 (Reapproved 1965). Papers treated according to the invention pass this test. There is no afterglow and the char length is less than 11.5 cm.

Alkylketene dimers have been tested by the U.S. Food and Drugs Authcrity and have been passed as acceptable for food wrapping paper additives as long as they are not present in quantities greater than 0.4% in the finished paper. This should be born in mind if the paper is to be used for food packaging.

The present invention will be described, by way of example only, with reference to the following formulations, in which the quantities are in parts by weight.

The pH of each formulation was adjusted to 8.0 by addition of sodium hydroxide.

Sheets of unsized handsheet paper, having a Cobb value of about 120 and no fire retardance were dipped into each formulation for about 1 second so that each sheet took up eponxraply the same weight of solution. The sheets were then dried and wsighed. The total weight uptake of selids for each sheet and its propertion are given below.

In each case the handsheet paper had no afterglow and did not char for more than 11.5 en. The sheet strengths were good and were not affected by the treioment .The appearance of the sheets is good, there being no browning to cryscalation, indicating the compatibilicy of the system.

The formulations were used in the treatment bath of a commercial paper making factory to treat continuous webs of paper, After hours use there was no evidence of any corrosion of the rollers.

All parts and perdentages herein are by .weight unless otherwise indicated. RTM indicates a registered trade mark.

## Claims

1. An aqueous paper-treating solution comprising from 10 to 70 parts of ionic fire-retardant material and from 0.2 tc 1 part of an alkylketene dimer, characterised in that,the solution has a pH from 7.8 to 8.2.

2. A solution according to claim 1, characterised in that,the pH is 8.0.

3. A solution according to claim 1 or 2, characterised in that, the alkylketene dimer is supplied as an aqueous emulsion containing about 6% alkylketene dimer, a cationic starch, and having a total solids content of about 7.6%, specific gravity of about 1.02 at 25⁰C, a viscosity from 25 to 100 centipoise at 25⁰C and a pH from 3.5 to 4.0.

4. A solution according to any one of the preceding claims, characterised in that the fire retardant material comprises from 45 to 55% diammonium hydrogen phosphate, the balance being ammonium sulphate.

5. A solution according to any one of the preceding claims, characterised in that, it comprises up to 30 parts of the fire retardant material.

6. A method of treating a web of paper to render it fire and water resistant, characterised in that, the paper is treated with a solution according to any one of the preceding claims and drying the paper, wherein the treatment is such that the dried paper has a dry loading of fire retardant from 10 to 50% and of water repellent of 0.4 to 1.0%.

7. Water and fire-resistant paper when made according to the method of claim 6.
